# EUROPEAN PATENT SPECIFICATION

(11) **EP 1 850 185 B1**
(45) Date of publication and mention of the grant of the patent: **19.01.2011**
(21) Application number: 07107052.8
(22) Date of filing: 26.04.2007
(51) Int. Cl.: G03G 5/05, G03G 5/06

(54) **Imaging member, method of imaging using it and method of making said imaging member**
Abbildungselement, Verfahren zur Bildherstellung und Herstellungsverfahren für diese Abbildungselement
Élément de formation d' images, méthode de formation d' images et procédés de fabrication de cet element de formation d'images

(30) Priority: 26.04.2006 US 795044 P; 17.07.2006 US 487887
(43) Date of publication of application: 31.10.2007
(73) Proprietor: Xerox Corporation, Rochester, New York 14644 (US)
(72) Inventor: Yanus, John F., Webster, NY 14580 (US); Silvestri, Markus Rudolf, Fairport, NY 14450 (US); Renfer, Dale S., Webster, NY 14580 (US); Dinh, Kenny-Tuan, Webster, NY 14580 (US); Hinckel, M. John, Rochester, NY 14609 (US); Goodbrand, H. Bruce, Hamilton Ontario L8P 4N9 (CA); Bender, Timothy P., Toronto Ontario M8Y 1E6 (CA)
(74) Representative: Jones, Helen M.M.

(56) References cited:
- US-A- 4 273 846
- US-A1- 2004 126 684
- US-A1- 2004 126 685
- US-A1- 2005 136 349

## Description

The present disclosure, in various exemplary embodiments, relates generally to electrophotographic imaging members and, more specifically, to layered photoreceptor structures having a charge transport layer comprising isomers of certain terphenyl diamines.

Electrophotographic imaging members, i.e. photoreceptors, typically include a photoconductive layer formed on an electrically conductive substrate. The photoconductive layer is an insulator in the dark so that electric charges can be retained on its surface. Upon exposure to light, the charge is dissipated.

An electrostatic latent image is formed on the photoreceptor by first uniformly depositing an electric charge over the surface of the photoconductive layer by one of the many known means in the art. The photoconductive layer functions as a charge storage capacitor with charge on its free surface and an equal charge of opposite polarity on the conductive substrate. A light image is then projected onto the photoconductive layer. The portions of the layer that are not exposed to light retain their surface charge. After development of the latent image with toner particles to form a toner image, the toner image is usually transferred to a receiving substrate, such as paper.

A photoreceptor usually comprises a supporting substrate, a charge generating layer, and a charge transport layer ("CTL"). For example, in a negative charging system, the photoconductive imaging member may comprise a supporting substrate, an electrically conductive layer, an optional charge blocking layer, an optional adhesive layer, a charge generating layer, a charge transport layer, and an optional protective or overcoat layer. In various embodiments, the charge transport layer may be one single layer or may comprise multiple layers having the same or different compositions at the same or different concentrations.

The charge transport layer usually comprises, at a minimum, charge transporting molecules ("CTMs") dissolved in a polymer binder resin, the layer being substantially non-absorbing in a spectral region of intended use, for example, visible light, while also being active in that the injection of photogenerated charges from the charge generating layer can be accomplished. Further, the charge transport layer allows for the efficient transport of charges to the free surface of the transport layer.

When a charge is generated in the charge generating layer, it should be efficiently injected into the charge transport molecule in the charge transport layer. The charge should also be transported across the charge transport layer in a short time, more specifically in a time period shorter than the time duration between the exposing and developing steps in an imaging device. The transit time across the charge transport layer is determined by the charge carrier mobility in the charge transport layer. The charge carrier mobility is the velocity per unit field and has dimensions of cm²/V·sec. The charge carrier mobility is generally a function of the structure of the charge transport molecule, the concentration of the charge transport molecule in the charge transport layer, and the electrically "inactive" binder polymer in which the charge transport molecule is dispersed.

The charge carrier mobility must be high enough to move the charges injected into the charge transport layer during the exposure step across the charge transport layer during the time interval between the exposure step and the development step. To achieve maximum discharge or sensitivity for a fixed exposure, the photoinjected charges must transit the transport layer before the imagewise exposed region of the photoreceptor arrives at the development station. To the extent the carriers are still in transit when the exposed segment of the photoreceptor arrives at the development station, the discharge is reduced and hence the contrast potentials available for development are also reduced. The transit time of charges across the charge transport layer and charge carrier mobility are related to each other by the expression transit time = (transport layer thickness)²/(mobility × applied voltage).

It is known in the art to increase the concentration of the charge transport molecule dissolved or molecularly dispersed in the binder. However, phase separation or crystallization sets an upper limit to the concentration of the transport molecules that can be dispersed in a binder. One way of increasing the solubility of the charge transport molecule is to attach long alkyl groups onto the transport molecules. However, these alkyl groups are "inactive" and do not transport charge. For a given concentration of charge transport molecule, a larger side chain can actually reduce the charge carrier mobility. A second factor that reduces the charge carrier mobility is the dipole content of the charge transport molecule in their side groups as well as that of the binder in which the molecules are dispersed.

One charge transport molecule known in the art is N,N'-diphenyl-N,N'-bis(3-methylphenyl)-[1,1'-biphenyl]-4,4'-diamine (TPD). TPD has a zero-field mobility of about 1.38 × 10⁻⁶ cm²/V·sec at a concentration of 40 weight percent in polycarbonate. Zero-field mobility µ₀ is the mobility extrapolated down to vanishing fields, i.e., the field E in µ =µ₀ exp(β·E^{0.5}) is set to zero. In general the field dependence expressed by β is weak.

There continues to be a need for an improved imaging member having a charge transport layer with high carrier charge mobility. Such an imaging member would allow for increases in the speed of imaging devices such as printers and copiers.

In U.S. Patent 4,273,846, to Pai et al., an imaging member having a charge transport layer containing a terphenyl diamine is described.

U.S. -A-2002-0077632, discloses aryldiamine charge transport molecules having more than 3 phenyl groups between the nitrogen atoms of the aryldiamine.

U.S. A-2004-0126684 ; U.S. Patent 7,005,222, to Horgan et al., and U.S. US-A-2005/0136349 disclose a plurality of charge transport layers which may contain a terphenyl diamine. The present invention relates to photoconductive imaging members having a charge transport layer comprising polymer binder and a charge transport component selected from certain terphenyl diamines. The imaging member of the invention is defined in claim 1, methods of imaging are claimed in claim 10 and methods of making the imaging member one defined in claim 11. Examples of these terphenyl diamines include isomers of N,N'-bis(methylphenyl)-N,N'-bis[4-(n-butyl)phenyl]-[p-terphenyl]-4,4"-diamine, having the structure of Formula (I): wherein R₁ is a methyl group (-CH₃) in the ortho, meta, or para position and R₂ is a butyl group (-C₄H₉). The photoconductive imaging members possess a number of the advantages illustrated herein including enhanced performance properties.

Also disclosed herein are methods of making such imaging members and methods of imaging utilizing such imaging members. The imaging members have improved carrier charge mobility and allow for imaging and printing at increased speeds.

In an embodiment, the imaging member has a charge generating layer and a charge transport layer comprising a polymer binder resin and the terphenyl diamines isomers noted above. The imaging member may be of a flexible belt design or a rigid drum design.

In another embodiment, the imaging member has a charge generating layer and a charge transport layer comprising two layers, a bottom layer and a top layer. The bottom layer and top layer are adjacent to each other and the bottom layer is adjacent to the charge generating layer. Both the bottom layer and the top layer comprise a polymer binder resin and a terphenyl diamine isomer selected from the group described above. The terphenyl diamine isomer in each layer may be the same or different. The concentration of the terphenyl diamine isomer in the bottom layer is greater than the concentration of the terphenyl diamine isomer in the top layer.

In still a further embodiment, a flexible imaging member is provided comprising a charge generating layer, and overlaid thereon and in contiguous contact therewith, a charge transport layer having two or more layers. The layers comprise one or more of the terphenyl diamines isomers shown above, wherein the concentration of the terphenyl diamine isomer is greater in the charge transport layer in contiguous contact with the charge generating layer.

In another embodiment, the imaging member has a charge generating layer and a charge transport layer comprising two layers, a bottom or first layer and a top or second layer. The bottom layer and top layer are adjacent to each other and the bottom layer is adjacent to the charge generating layer. Both the bottom layer and the top layer comprise a polymer binder resin and a terphenyl diamine isomer from the group described above. The terphenyl diamine isomer in each layer may be the same or different. The bottom layer comprises from about 30 weight percent to about 50 weight percent of its terphenyl diamine isomer and the top layer comprises from about 0 weight percent to about 45 weight percent of its terphenyl diamine isomer, the top layer having a lower concentration of its terphenyl diamine isomer than the bottom layer.

These and other non-limiting features or characteristics of the present disclosure will be further described below.

The following is a brief description of the drawings, which are presented for the purposes of illustrating the exemplary embodiments disclosed herein and not for the purposes of limiting the same.
**Fig. 1** is a cross-sectional view of an exemplary embodiment of an imaging member having a single charge transport layer.
**Fig. 2** is a cross-sectional view of another exemplary embodiment in which the imaging member has a dual-layer charge transport layer.
**Fig. 3** is a graph showing the mobility vs. field strength of three exemplary embodiments of the present disclosure against a control.
**Fig. 4** is a PIDC graph of three exemplary embodiments of the present disclosure against a control.
**Fig. 5A** is a PIDC graph of three exemplary embodiments of the present disclosure after 10,000 exposures and discharges.
**Fig. 5B** is the same as **Fig. 5A****,** but over a different range.
**Fig. 6** is a graph showing the change in mobility with concentration of the charge transport molecule in exemplary embodiments of the present disclosure.
**Fig. 7** is a graph showing the difference in potential of two temperatures for an exemplary embodiment of the present disclosure.

The imaging members disclosed herein can be used in a number of different known imaging and printing processes including, for example, electrophotographic imaging processes, especially xerographic imaging and printing processes wherein charged latent images are rendered visible with toner compositions of an appropriate charge polarity. Moreover, the imaging members of this disclosure are also useful in color xerographic applications, particularly high-speed color copying and printing processes.

The exemplary embodiments of this disclosure are more particularly described below with reference to the drawings. Although specific terms are used in the following description for clarity, these terms are intended to refer only to the particular structure of the various embodiments selected for illustration in the drawings and not to define or limit the scope of the disclosure. The same reference numerals are used to identify the same structure in different Figures unless specified otherwise. The structures in the Figures are not drawn according to their relative proportions and the drawings should not be interpreted as limiting the disclosure in size, relative size, or location. In addition, though the discussion will address negatively charged systems, the imaging members of the present disclosure may also be used in positively charged systems.

An exemplary embodiment of the imaging member of the present disclosure is illustrated in **FIGURE 1****.** The substrate **32** has an optional conductive layer **30.** An optional hole blocking layer **34** can also be applied, as well as an optional adhesive layer **36.** The charge generating layer **38** is located between the optional adhesive layer **36** and the charge transport layer **40.** An optional ground strip layer **41** operatively connects the charge generating layer **38** and the charge transport layer **40** to the conductive layer **30.** An opposite anti-curl back layer **33** may be applied to the side of the substrate **32** opposite from the electrically active layers. An optional overcoat layer **42** may be placed upon the charge transport layer **40.**

In another exemplary embodiment as illustrated in **FIGURE 2****,** the charge transport layer comprises dual layers **40B** and **40T.** The dual layers **40B** and **40T** may have the same or different compositions. In other embodiments, a plurality of charge transport layers can be utilized, although not shown in the figures.

The charge transport layer **40** of **Figure 1** comprises certain specific charge transport materials which are capable of supporting the injection of photogenerated holes or electrons from the charge generating layer **38** and allowing their transport through the charge transport layer to selectively discharge the surface charge on the imaging member surface. The charge transport layer, in conjunction with the charge generating layer, should also be an insulator to the extent that an electrostatic charge placed on the charge transport layer is not conducted in the absence of illumination. It should also exhibit negligible, if any, discharge when exposed to a wavelength of light useful in xerography, e.g., about 400 to 900 nm. This ensures that when the imaging member is exposed, most of the incident radiation is used in the charge generating layer beneath it to efficiently produce photogenerated charges.

The charge transport layer of the present disclosure comprises specific charge transport molecules which support the injection and transport of photogenerated holes or electrons. The charge transport molecules have the molecular structure shown in Formula (I): wherein R₁ is a methyl group (-CH₃) in the ortho, meta, or para position and R₂ is a butyl group (-C₄H₉).

The full name for this charge transport molecule is N,N'-bis(x-methylphenyl)-N,N'-bis[4-(n-butyl)phenyl]-[p-terphenyl]-4,4"-diamine, where x is 2, 3, or 4, corresponding to the ortho, meta, or para isomers. In this disclosure, this charge transport molecule will be referred to as "methyl terphenyl" or "MeTer" and the ortho, meta, and para embodiments will be referred to as o-methyl terphenyl ("o-MeTer"), m-methyl terphenyl ("m-MeTer"), and p-methyl terphenyl ("p-MeTer"), respectively. When referring to all three of the isomers as a group, they will be referred to as "the methyl terphenyl compounds".

In a specific embodiment, a charge transport molecule is p-methyl terphenyl having the molecular structure shown in Formula (II):

In another specific embodiment, a charge transport molecule is o-methyl terphenyl having the molecular structure shown in Formula (III):

In another specific embodiment, a charge transport molecule is m-methyl terphenyl having the molecular structure shown in Formula (IV):

Although the properties of the three methyl terphenyl compounds were expected to be equivalent, the p-methyl terphenyl isomer of Formula (II) has been unexpectedly found to possess several advantageous properties over the other two isomers. It was expected that the carrier charge mobilities of all three methyl terphenyl isomers would be about equivalent. However, the para isomer had a mobility 50% higher than the other two isomers. In addition, it was expected that temperature changes would equally affect the mobility of the three isomers. However, the para isomer exhibited less sensitivity to temperature changes.

If desired, the charge transport layer may also comprise other charge transport molecules. For example, the charge transport layer may contain other triarylamines such as TPD, tri-p-tolylamine, 1,1-bis(4-di-p-tolylaminophenyl) cyclohexane, and other similar triarylamines. The additional charge transport molecules may, e.g., help minimize background voltage. In particular, embodiments where one of the three methyl terphenyl compounds is mixed with TPD are contemplated. The present disclosure also contemplates mixtures of the three methyl terphenyl isomers, especially mixtures containing p-methyl terphenyl.

The charge transport layer also comprises a polymer binder resin in which the charge transport molecules or components are dispersed. The resin should be substantially soluble in a number of solvents, like methylene chloride or other solvent so that the charge transport layer can be coated onto the imaging member. Typical binder resins soluble in methylene chloride include polycarbonate resin, polyvinylcarbazole, polyester, polyarylate, polyacrylate, polyether, polysulfone, polystyrene, polyamide, Molecular weights of the binder resin can vary from, for example, about 20,000 to about 300,000, including about 150,000.

Polycarbonate resins having a weight average molecular weight Mw, of from about 20,000 to about 250,000 are suitable for use, and in embodiments from about 50,000 to about 120,000, may be used. The electrically inactive resin material may include poly(4,4'-dipropylidene-diphenylene carbonate) with a weight average molecular weight (M_{w}) of from about 35,000 to about 40,000, available as LEXAN 145 from General Electric Company; poly(4,4'-isopropylidene-diphenylene carbonate) with a molecular weight of from about 40,000 to about 45,000, available as LEXAN 141 from the General Electric Company; and a polycarbonate resin having a molecular weight of from about 20,000 to about 50,000 available as MERLON from Mobay Chemical Company. Resins known as PC-Z®, available from Mitsubishi Gas Chemical Corporation, may also be used. In specific embodiments, MAKROLON, available from Bayer Chemical Company, and having a molecular weight of from about 70,000 to about 200,000, is used. Methylene chloride is used as a solvent in the charge transport layer coating mixture for its low boiling point and the ability to dissolve charge transport layer coating mixture components to form a charge transport layer coating solution.

The charge transport layer of the present disclosure in embodiments comprises from about 25 weight percent to about 60 weight percent of the charge transport molecules and from about 40 weight percent to about 75 weight percent by weight of the polymer binder resin, both by total weight of the charge transport layer. In specific embodiments, the charge transport layer comprises from about 40 weight percent to about 50 weight percent of the charge transport molecules and from about 50 weight percent to about 60 weight percent of the polymer binder resin.

In embodiments where the charge transport layer comprises dual or multiple layers, the layers may differ in the charge transport molecules selected, the polymer binder resin selected, both or neither. However, generally the charge transport molecule(s) and polymer binder resin are the same and the dual or multiple layers differ only in the concentration of the charge transport molecule(s). More specifically, the top layer has a lower concentration of charge transport molecule(s) than the bottom layer. In further embodiments, the bottom layer comprises from about 30 weight percent to about 50 weight percent of the charge transport molecule(s) and the top layer comprises from about 0 weight percent to about 45 weight percent of the charge transport molecule(s), wherein the weight percentage is based on the weight of the respective layer, not the total charge transport layer. In specific embodiments, the bottom layer comprises from about 30 weight percent to about 50 weight percent of the charge transport molecule(s) and the top layer comprises from about 25 weight percent to about 45 weight percent of the charge transport molecule(s). In further specific embodiments, the bottom layer comprises about 50 weight percent of all charge transport molecules and the top layer comprises about 40 weight percent of all charge transport molecules. Generally, the concentration of the selected methyl terphenyl molecule is greater in the bottom layer than the top layer. If the bottom layer has a different methyl terphenyl molecule than that of the top layer, the concentration of the methyl terphenyl molecule in the bottom layer should greater than or equal to the concentration of the methyl terphenyl molecule in the top layer.

In embodiments having a single charge transport layer, the charge transport molecule(s) is substantially homogenously dispersed throughout the polymer binder. In embodiments where the charge transport layer comprises dual layers, the charge transport molecule(s) in the bottom layer is substantially homogeneously dispersed throughout the bottom layer and the charge transport molecule(s) in the top layer is substantially homogeneously dispersed throughout the top layer.

Generally, the thickness of the charge transport layer is from about 10 to about 100 micrometers, including from about 20 micrometers to about 60 micrometers, but thicknesses outside these ranges can also be used. In general, the ratio of the thickness of the charge transport layer to the charge generating layer is in embodiments from about 2:1 to 200:1 and in some instances from about 2:1 to about 400:1. In specific embodiments, the charge transport layer is from about 10 micrometers to about 40 micrometers thick.

Any suitable technique may be used to mix and apply the charge transport layer onto the charge generating layer. Generally, the components of the charge transport layer are mixed into an organic solvent to form a coating solution. Typical solvents comprise methylene chloride, toluene, tetrahydrofuran, Typical application techniques include extrusion die coating, spraying, roll coating, wire wound rod coating, Drying of the coating solution may be effected by any suitable conventional technique such as oven drying, infra red radiation drying, air drying When the charge transport layer comprises dual or multiple layers, each layer is solution coated, then completely dried at elevated temperatures prior to the application of the next layer.

If desired, other known components may be added the charge transport layer or, if there are dual or multiple layers, to all of the layers. Such components may include antioxidants, such as a hindered phenol, leveling agents, surfactants, and light shock resisting or reducing agents. Particle dispersions may increase the mechanical strength of the charge transport layer as well.

The imaging member of the present disclosure may comprise a substrate **32,** optional anti-curl back layer **33,** an optional conductive layer **30** if the substrate is not adequately conductive, optional hole blocking layer **34,** optional adhesive layer **36,** charge generating layer **38,** charge transport layer **40,** an optional ground strip layer **41,** and an optional overcoat layer **42.** The remaining layers will now be described with reference to **Figs. 1-2****.**

The substrate support **32** provides support for all layers of the imaging member. Its thickness depends on numerous factors, including mechanical strength, flexibility, and economical considerations; the substrate for a flexible belt may, for example, be from about 50 micrometers to about 150 micrometers thick, provided there are no adverse effects on the final electrophotographic imaging device. The substrate support is not soluble in any of the solvents used in each coating layer solution, is optically transparent, and is thermally stable up to a high temperature of about 150°C. A typical substrate support is a biaxially oriented polyethylene terephthalate. Another suitable substrate material is a biaxially oriented polyethylene naphtahlate, having a thermal contraction coefficient ranging from about 1 x 10⁻⁵/°C to about 3 x 10⁻⁵/°C and a Young's Modulus of from about 5 x 10⁵ psi to about 7 x 10⁵ psi (3.4 x 10⁹ to 4.8 x 10⁹ Pa). However, other polymers are suitable for use as substrate supports. The substrate support may also be made of a conductive material, such as aluminum, chromium, nickel, brass Again, the substrate support may flexible or rigid, seamed or seamless, and have any configuration, such as a plate, drum, scroll, belt,

The optional conductive layer **30** is present when the substrate support 32 is not itself conductive. It may vary in thickness depending on the optical transparency and flexibility desired for the electrophotographic imaging member. Accordingly, when a flexible electrophotographic imaging belt is desired, the thickness of the conductive layer may be from about 2 to 75 nm, and more specifically from about 5 to 20 nm for an optimum combination of electrical conductivity, flexibility and light transmission. The conductive layer may be formed on the substrate by any suitable coating technique, such as a vacuum depositing or sputtering technique. Typical metals suitable for use as the conductive layer include aluminum, zirconium, niobium, tantalum, vanadium, hafnium, titanium, nickel, stainless steel, chromium, tungsten, molybdenum,

The optional hole blocking layer **34** forms an effective barrier to hole injection from the adjacent conductive layer into the charge generating layer. Examples of hole blocking layer materials include gamma amino propyl triethoxyl silane, zinc oxide, titanium oxide, silica, polyvinyl butyral, phenolic resins, Hole blocking layers of nitrogen containing siloxanes or nitrogen containing titanium compounds are disclosed, for example, in U.S. Patent No. 4,291,110, U.S. Patent No. 4,338,387, U.S. Patent No. 4,286,033 and U.S. Patent No. 4,291,110. The blocking layer may be applied by any suitable conventional technique such as spraying, dip coating, draw bar coating, gravure coating, silk screening, air knife coating, reverse roll coating, vacuum deposition, chemical treatment The blocking layer should be continuous and more specifically have a thickness of from about 0.2 to about 2 micrometers.

An optional adhesive layer **36** may be applied to the hole blocking layer. Any suitable adhesive layer may be utilized. Any adhesive layer employed should be continuous and, more specifically, have a dry thickness from about 200 micrometers to about 900 micrometers and, even more specifically, from about 400 micrometers to about 700 micrometers. Any suitable solvent or solvent mixtures may be employed to form a coating solution for the adhesive layer. Typical solvents include tetrahydrofuran, toluene, methylene chloride, cyclohexanone, and mixtures thereof. Any other suitable and conventional technique may be used to mix and thereafter apply the adhesive layer coating mixture to the hole blocking layer. Typical application techniques include spraying, dip coating, roll coating, wire wound rod coating, Drying of the deposited coating may be effected by any suitable conventional technique such as oven drying, infra red radiation drying, air drying.

Any suitable charge generating layer **38** may be applied which can thereafter be coated over with a contiguous charge transport layer. The charge generating layer generally comprises a charge generating material and a film-forming polymer binder resin. Charge generating materials such as vanadyl phthalocyanine, metal free phthalocyanine, benzimidazole perylene, amorphous selenium, trigonal selenium, selenium alloys such as selenium-tellurium, selenium-tellurium-arsenic, selenium arsenide, and mixtures thereof may be appropriate because of their sensitivity to white light. Vanadyl phthalocyanine, metal free phthalocyanine and tellurium alloys are also useful because these materials provide the additional benefit of being sensitive to infrared light. Other charge generating materials include quinacridones, dibromo anthanthrone pigments, benzimidazole perylene, substituted 2,4-diamino-triazines, polynuclear aromatic quinones, Benzimidazole perylene compositions are well known and described, for example, in U.S. Patent No. 4,587,189, . Other suitable charge generating materials known in the art may also be utilized, if desired. The charge generating materials selected should be sensitive to activating radiation having a wavelength from about 600 to about 700 nm during the imagewise radiation exposure step in an electrophotographic imaging process to form an electrostatic latent image. In specific embodiments, the charge generating material is hydroxygallium phthalocyanine (OHGaPC) or oxytitanium phthalocyanine (TiOPC).

Any suitable inactive film forming polymeric material may be employed as the binder in the charge generating layer **38**, including those described, for example, in U.S. Patent No. 3,121,006. Typical organic polymer binders include thermoplastic and thermosetting resins such as polycarbonates, polyesters, polyamides, polyurethanes, polystyrenes, polyarylethers, polyarylsulfones, polybutadienes, polysulfones, polyethersulfones, polyethylenes, polypropylenes, polyimides, polymethylpentenes, polyphenylene sulfides, polyvinyl butyral, polyvinyl acetate, polysiloxanes, polyacrylates, polyvinyl acetals, polyamides, polyimides, amino resins, phenylene oxide resins, terephthalic acid resins, epoxy resins, phenolic resins, polystyrene and acrylonitrile copolymers, polyvinylchloride, vinylchloride and vinyl acetate copolymers, acrylate copolymers, alkyd resins, cellulosic film formers, poly(amideimide), styrene-butadiene copolymers, vinylidenechloride-vinylchloride copolymers, vinylacetate-vinylidenechloride copolymers, styrene-alkyd resins,

The charge generating material can be present in the polymer binder composition in various amounts. Generally, from about 5 to about 90 percent by volume of the charge generating material is dispersed in about 10 to about 95 percent by volume of the polymer binder, and more specifically from about 20 to about 50 percent by volume of the charge generating material is dispersed in about 50 to about 80 percent by volume of the polymer binder.

The charge generating layer generally ranges in thickness of from about 0.1 micrometer to about 5 micrometers, and more specifically has a thickness of from about 0.3 micrometer to about 3 micrometers. The charge generating layer thickness is related to binder content. Higher polymer binder content compositions generally require thicker layers for charge generation. Thickness outside these ranges can be selected in order to provide sufficient charge generation.

An optional anti-curl back coating **33** can be applied to the back side of the substrate support **32** (which is the side opposite the side bearing the electrically active coating layers) in order to render flatness. Although the anti-curl back coating may include any electrically insulating or slightly conductive organic film forming polymer, it is usually the same polymer as used in the charge transport layer polymer binder. An anti-curl back coating from about 7 to about 30 micrometers in thickness is found to be adequately sufficient for balancing the curl and render imaging member flatness.

An electrophotographic imaging member may also include an optional ground strip layer **41.** The ground strip layer comprises, for example, conductive particles dispersed in a film forming binder and may be applied to one edge of the photoreceptor to operatively connect charge transport layer **40,** charge generating layer **38,** and conductive layer **30** for electrical continuity during electrophotographic imaging process. The ground strip layer may comprise any suitable film forming polymer binder and electrically conductive particles. Typical ground strip materials include those enumerated in U.S. Patent No. 4,664,995. The ground strip layer **41** may have a thickness from about 7 micrometers to about 42 micrometers, and more specifically from about 14 micrometers to about 23 micrometers.

An overcoat layer **42,** if desired, may be utilized to provide imaging member surface protection as well as improve resistance to abrasion. Overcoat layers are known in the art. Generally, they serve a function of protecting the charge transport layer from mechanical wear and exposure to chemical contaminants.

The imaging member formed may have a rigid drum configuration or a flexible belt configuration. The belt can be either seamless or seamed. In this regard, the fabricated multilayered flexible photoreceptors of the present disclosure may be cut into rectangular sheets and converted into photoreceptor belts. The two opposite edges of each photoreceptor cut sheet are then brought together by overlapping and may be joined by any suitable means including ultrasonic welding, gluing, taping, stapling, and pressure and heat fusing to form a continuous imaging member seamed belt, sleeve, or cylinder. The prepared imaging member may then be employed in any suitable and conventional electrophotographic imaging process which utilizes uniform charging prior to imagewise exposure to activating electromagnetic radiation. When the imaging surface of an electrophotographic member is uniformly charged with an electrostatic charge and imagewise exposed to activating electromagnetic radiation, conventional positive or reversal development techniques may be employed to form a marking material image on the imaging surface of the electrophotographic imaging member of this disclosure. Thus, by applying a suitable electrical bias and selecting toner having the appropriate polarity of electrical charge, one may form a toner image in the charged areas or discharged areas on the imaging surface of the electrophotographic member of the present disclosure.

The imaging members of the present disclosure may be used in imaging. This method comprises generating an electrostatic latent image on the imaging member. The latent image is then developed and transferred to a suitable substrate, such as paper. Processes of imaging, especially xerographic imaging and printing, including digital, are also encompassed by the present disclosure. More specifically, the layered photoconductive imaging members of the present development can be selected for a number of different known imaging and printing processes including, for example, electrophotographic imaging processes, especially xerographic imaging and printing processes wherein charged latent images are rendered visible with toner compositions of an appropriate charge polarity. Moreover, the imaging members of this disclosure are useful in color xerographic applications, particularly high-speed color copying and printing processes and which members are in embodiments sensitive in the wavelength region of, for example, from about 500 to about 900 nanometers, and in particular from about 650 to about 850 nanometers, thus diode lasers can be selected as the light source.

The present disclosure will further be illustrated in the following non-limiting working examples, it being understood that these examples are intended to be illustrative only and that the disclosure is not intended to be limited to the materials, conditions, process parameters recited herein. All proportions are by weight unless otherwise indicated.

### EXAMPLES

### Example 1 - Preparation of Specific Terphenyl Diamines

### A) Preparation of N,N'-bis(3-methylphenyl)-N,N'-bis[4-(n-butyl)phenyl]-[p-terphenyl]-4,4"-diamine, or m-methyl terphenyl (m-MeTer)

A 250 ml three necked round bottom flask equipped with a mechanical stirrer and purged with argon was charged with 14.34 grams (0.06 moles) of 3-methylphenyl-[4-(n-butyl)phenyl]amine, 9.64 grams (0.02 moles) of 4,4"-diiodoterphenyl, 15 grams (0.11 moles) of potassium carbonate, 10 grams of copper bronze and 50 milliliters of C₁₃ -C₁₅ aliphatic hydrocarbons, i.e. Soltrol® 170 (Phillips Chemical Company). The mixture was heated for 18 hours at 210º C. The product was isolated by the addition of 200 mls of n-octane and hot filtered to remove inorganic solids. The product crystallized out on cooling and was isolated by filtration. Treatment with alumina yielded substantially pure, about 99 percent m-methyl terphenyl (m-MeTer) in approximately 75% yield.

### B) Preparation of N,N'-bis(4-methylphenyl)-N,N'-bis[4-(n-butyl)phenyl]-[p-terphenyl]-4,4"-diamine, or p-methyl terphenyl (p-MeTer)

P-methyl terphenyl (p-MeTer) was prepared in the same manner as m-methyl terphenyl above, except that the 3-methylphenyl-[4-(n-butyl)phenyl]amine was replaced with 4-methylphenyl-[4-(n-butyl)phenyl]amine.

### C) Preparation of N,N'-bis(2-methylphenyl)-N,N'-bis[4-(n-butyl)phenyl]-[p-terphenyl]-4,4"-diamine, or o-methyl terphenyl (o-MeTer)

O-methyl terphenyl (o-MeTer) was prepared in the same manner as m-methyl terphenyl above, except that the 3-methylphenyl-[4-(n-butyl)phenyl]amine was replaced with 2-methylphenyl-[4-(n-butyl)phenyl]amine.

### Example 2 - Preparation of imaging member (Reference)

An electrophotographic imaging member web stock was prepared by providing a 0.02 micrometer thick titanium layer coated on a biaxially oriented polyethylene naphthalate substrate (KADALEX, available from ICI Americas, Inc.) having a thickness of 89 micrometers (3.5 mils) and applying thereto, using a gravure coating technique and a solution containing 10 grams gamma aminopropyltriethoxysilane, 10.1 grams distilled water, 3 grams acetic acid, 684.8 grams of 200 proof denatured alcohol and 200 grams heptane. This layer was then allowed to dry for 5 minutes at 135°C in a forced air oven. The resulting blocking layer had an average dry thickness of 0.05 micrometer measured with an ellipsometer.

An adhesive interface layer was then prepared by applying with extrusion process to the blocking layer a wet coating containing 5 percent by weight based on the total weight of the solution of polyester adhesive (MOR-ESTER 49,000, available from Morton International, Inc.) in a 70:30 volume ratio mixture of tetrahydrofuran:cyclohexanone. The adhesive interface layer was allowed to dry for 5 minutes at 135°C in a forced air oven. The resulting adhesive interface layer had a dry thickness of 0.065 micrometer

The adhesive interface layer was thereafter coated with a charge generating layer. The charge generating layer dispersion was prepared by introducing 0.45 grams of LUPILON 200 (PC-Z 200) available from Mitsubishi Gas Chemical Corp and 50ml of tetrahydrofuran into a 100 ml glass bottle. To this solution was added 2.4 grams of hydroxygallium phthalocyanine and 300 grams of 3.2 mm (1/8 inch) diameter stainless steel shot. This mixture was then placed on a ball mill for 20 to 24 hours. Subsequently, 2.25 grams of PC-Z 200 was dissolved in 46.1 gm of tetrahydrofuran, then added to this OHGaPc slurry. This slurry was then placed on a shaker for 10 minutes. The resulting slurry was, thereafter, coated onto the adhesive interface by an extrusion application process to form a layer having a wet thickness of 6 µm (0.25 mil). However, a strip about 10 mm wide along one edge of the substrate web bearing the blocking layer and the adhesive layer was deliberately left uncoated by any of the charge generating layer material to facilitate adequate electrical contact by the ground strip layer that is applied later. This charge generating layer was dried at 135°C for 5 minutes in a forced air oven to form a dry charge generating layer having a thickness of 0.4 micrometer layer.

A charge transport layer coating solution was then prepared. In a one ounce bottle, 1.3 grams of MAKROLON was dissolved in 11 grams of methylene chloride. 1.07 grams of p-methyl terphenyl (p-MeTer) was stirred in until a complete solution was achieved. A charge transport layer was coated onto the charge generating layer using a 100 µm (4 mil) Bird bar. The layer was dried at 40-100°C for 30 minutes in a forced air oven to yield a first imaging member having a charge transport layer that was 25 µm thick and contained 40 weight percent of p-methyl terphenyl (p-MeTer) and 60 weight percent MAKROLON.

A second imaging member was made as above, except that 1.07 grams of m-methyl terphenyl (m-MeTer) was stirred into the solution. The result was an imaging member having a charge transport layer that was 25 µm thick and contained 40 weight percent m-methyl terphenyl (m-MeTer) and 60 weight percent MAKROLON.

A third imaging member was made as described for the first imaging member above, except that 1.07 grams of o-methyl terphenyl (o-MeTer) was stirred into the solution. The result was an imaging member having a charge transport layer that was 25 µm thick and contained 40 weight percent of o-methyl terphenyl (o-MeTer) and 60 weight percent MAKROLON.

### Experimental Data

Four imaging members were provided with charge transport layers containing 40 weight percent TPD, 40 weight percent p-methyl terphenyl (p-MeTer), 40 weight percent m-methyl terphenyl (m-MeTer), and 40 weight percent o-methyl terphenyl (o-MeTer), respectively. The remaining 60 weight percent of each imaging member was MAKROLON. The 40 weight percent TPD served as control. The imaging members were exposed to different electric fields and their mobilities were measured. The resulting data is shown in Table 1 below and in **Fig. 3**, which is a graph of the results showing mobility vs. electric field strength.

**Table 1**

| **Sample ID** | **40% TPD** | **40% p-MeTer** | **40% m-MeTer** | **40% o-MeTer** |
|---|---|---|---|---|
| Thickness of CTL (µm) | 25.5 | 25.3 | 25:4 | 24.9 |
| Bias (V) | Transit Time (ms) | Transit Time (ms) | Transit Time (ms) | Transit Time (ms) |
| 50 V | 70.70 | 10.01 | 14.62 | 15.18 |
| 70 V | 49.90 | 7.15 | 9.66 | 9.75 |
| 100 V | 30.75 | 4.47 | 6.23 | 6.38 |
| 140 V | 20.75 | 3.04 | 4.15 | 4.39 |
| 180 V | 14.54 | 2.31 | 3.04 | 3.12 |
| 250 V | 9.90 | 1.60 | 2.05 | 2.14 |
| 350 V | 6.19 | 1.04 | 1.35 | 1.43 |
| 500 V | 3.83 | 0.68 | 0.88 | 0.92 |
| Measured Zero Field Mobility µ₀ (cm²/V·s) | 1.38 x 10^{- 6} | 1.07 x 10⁻⁵ | 7.33 x 10⁻⁶ | 6.95 x 10⁻⁶ |
| Field parameter β in µ =µ₀ ·exp(β·E^{0.5}) ((cm/V)^{0.5}) | 2.09 x 10^{- 3} | 1.31 x 10⁻³ | 1.65 x 10⁻³ | 1.55 x 10⁻³ |
| Activation energy from Arrhenius plot of the initial discharge speed (eV) | 376 | 274 | 326 | N/A |

The unexpected results of this test indicated that the three methyl terphenyl compounds did not have the same mobilities, the same field parameters, and the same activation energies. Higher mobility has the advantage of faster transport. The lower the field parameter, the less undesirable electrostatic spreading and the take place. The activation energy governs the temperature dependence, and again, the lower, the better, since it makes the photoreceptor less susceptible to temperature variations in the environment.

Next, the xerographic electrical properties of the four imaging members were measured. Each member was charged to an initial value of -500V, then discharged, to obtain a photoinduced discharge curve (PIDC) for each imaging member. The PIDCs are shown in **Fig. 4****.** The photosensitivity of an imaging member is usually provided in terms of the amount of exposure energy in ergs/cm², designated as E_{1/2}, required to achieve 50 percent photodischarge from V_{ddp} to half of its initial value (1 ergs/cm² is 10⁻³ Jm⁻²). The higher the photosensitivity is, the smaller the E_{1/2} value is. While all three of the methyl terphenyl compounds showed higher photosensitivity than TPD, p-methyl terphenyl (p-MeTer) showed the greatest photosensitivity of the three methyl terphenyl compounds. p-methyl terphenyl also performed better than TPD across the entire range.

Thereafter, tests were performed in which imaging members were first exposed and discharged 10,000 times, and the PIDCs were then measured to determine the deterioration in performance. These tests were performed on three imaging members for each of the 40 weight percent TPD, 40 weight percent p-MeTer, and 40 weight percent m-MeTer charge transport layers and on one imaging member for the 40 weight percent o-MeTer charge transport layer. The results are shown in **Fig. 5A****,** which compares the fatigued PIDCs for the members that were been discharged 10,000 times against the PIDCs of **Fig. 4****.** **Fig. 5B** shows the same results as **Fig. 5A**, but over a shorter range of exposure. One notable result was that the performance of the charge transport layer containing p-MeTer deteriorated significantly less than the charge transport layers containing m-MeTer and o-MeTer. The performance of the charge transport layer containing p-MeTer deteriorated about 15% less than the charge transport layer containing m-MeTer and deteriorated about 49% less than the charge transport layer containing o-MeTer. Table 2 summarizes the data depicted in **Fig. 5**.

**Table 2**

| **CTM** | **Condition** | **Potential (V) @ 10 ergs/cm²** | **Δ** | **Initial Slope (V·erg/cm²) @ -500V** | **Δ** | **E_{1/2} (erg/cm²)** | **Δ** |
|---|---|---|---|---|---|---|---|
| TPD | Initial | 50 | 60 | 262 | 19 | 1.05 | 0.26 |
| | Fatigued | 110 | | 243 | | 1.32 | |
| p-MeTer | Initial | 36 | 41 | 332 | 7 | 0.83 | 0.13 |
| | Fatigued | 77 | | 325 | | 0.96 | |
| m-MeTer | Initial | 62 | 47 | 312 | 2 | 0.92 | 0.20 |
| | Fatigued | 109 | | 310 | | 1.12 | |
| o-MeTer | Initial | 71 | 62 | 322 | 1 | 0.89 | 0.30 |
| | Fatigued | 133 | | 321 | | 1.19 | |

Three imaging members containing 30 weight percent, 40 weight percent, and 50 weight percent m-MeTer in their respective charge transport layer were fabricated. These imaging members were exposed to different electric fields and their mobilities were measured. The results are shown in **Fig. 6**. As noted, mobility increased as the concentration of the charge transport molecule was increased.

An imaging member with 40 weight percent p-MeTer in the charge transport layer and an imaging member with 40 weight percent TPD were fabricated. They were exposed at 35ºC and at 25ºC and the voltage remaining on the photoreceptor after exposure was measured. Normally, the voltage remaining on the photoreceptor after exposure for a given exposure-to-measurement time varies with the temperature. However, this effect was not observed in p-MeTer for the relevant times. This can be very useful in a printing machine, which can operate in a broad temperature range (e.g. from 15-40ºC), because the latent image on the photoconductor is less susceptible to local temperature variation across the photoconductor within the print engine. Unlike TPD, all charges transited the p-MeTer charge transport layer at the relevant temperatures in similar times, making the photoreceptor insensitive to temperature variations. **Fig. 7** shows the results of this experiment. The difference in the potentials at 25ºC and 35ºC were plotted against time. p-MeTer showed only small changes in the discharge potential in contrast to TPD.

## Claims

1. An imaging member comprising at least one charge transport layer comprising a polymer binder resin and a first and a second charge transport component, wherein one of the charge transport components is a terphenyl diamine charge transport component comprised of an isomer of N,N'-bis(methylphenyl)-N,N'-bis[4-(n-butyl)phenyl]-[p-terphenyl]-4,4"-diamine of Formula (I): wherein R₁ is a methyl group (-CH₃) in the ortho, meta, or para position and R₂ is a butyl group (-C₄H₉), **characterised in that** the first charge transport component and the second charge transport component are different isomers of N,N'-bis(methylphenyl)-N,N'-bis[4-(n-butyl)phenyl]-[p-terphenyl]-4,4"-diamine.

2. The imaging member of claim 1, wherein the charge transport component comprises an isomer selected from
i) N,N'-bis(2-methylphenyl)-N,N^{'}-bis[4-(n-butyl)phenyl]-[p-terphenyl]-4,4"-diamine;
ii) N,N'-bis(3-methylphenyl)-N,N'-bis[4-(n-butyl)phenyl]-[p-terphenyl]-4,4"-diamine; and
iii) N,N'-bis(4-methylphenyl)-N,N'-bis[4-(n-butyl)phenyl]-[p-terphenyl]-4,4"-diamine.

3. The imaging member of any preceding claim, wherein the terphenyl diamine comprises from 25 weight percent to 60 weight percent of the charge transport layer, based on the total weight of the charge transport layer, preferably from 40 weight percent to 50 weight percent.

4. The imaging member of any preceding claim, wherein the binder is selected from the group consisting of polyesters, polyvinyl butyrals, polycarbonates, polystyrene, and polyvinyl formats.

5. The imaging member of claim 4, wherein the binder is a polycarbonate selected from the group consisting of poly(4,4'-isopropyliene diphenyl carbonate), poly(4,4'-diphenyl-1,1'cyclohexane carbonate), or a polymer blend thereof.

6. The imaging member of claim 1, wherein the total thickness of the charge transport layer is from 10 µm to 100 µm, preferably from 20 µm to 60 µm.

7. An imaging member according to claim 1, comprising a substrate, an optional conductive layer, an optional hole blocking layer, an optional adhesive layer, a charge generating layer, and the at least one charge transport layer,
wherein the charge transport layer comprises a bottom layer and a top layer; wherein the bottom and top layers each comprise a polymer binder resin and a terphenyl diamine of formula I, and
wherein the bottom layer comprises from 30 weight percent to 50 weight percent of the terphenyl diamine and the top layer comprises from 0 weight percent to 45 weight percent of the terphenyl diamine, the top layer having a lower concentration of the terphenyl diamine than the bottom layer.

8. The imaging member of claim 7, wherein the supporting substrate, which optionally comprises a conductive surface layer, is selected from the group consisting of copper, brass, nickel, zinc, chromium, stainless steel, conductive plastics, conductive rubbers, aluminum, semitransparent aluminum, steel, cadmium, silver, gold, zirconium, niobium, tantalum, vanadium, hafnium, titanium, tungsten, molybdenum, indium, tin and metal oxides.

9. A method of imaging, comprising:
generating an electrostatic latent image on an imaging member;
developing the latent image; and
transferring the developed electrostatic image to a suitable substrate;
wherein the imaging member has a charge transport layer comprising first and second charge transport components, wherein one of the charge transport components is a terphenyl diamine having the structure of Formula (I): wherein R₁ is a methyl group in the ortho, meta, or para position and R₂ is a butyl group, the first charge transport component and the second charge transport component are different isomers of N,N'-bis(methylphenyl)-N,N'-bis[4-(n-butyl)phenyl]-[p-terphenyl]-4,4"-diamine.

10. A method of making an imaging member according to claim 1, in which a substrate is coated with a coating composition comprising the resin, the terphenyl diamine isomers and a solvent in which the resin is soluble, and the composition is dried.

## Patentansprüche

1. Bilderzeugungselement umfassend wenigstens eine Ladungstransportschicht umfassend ein polymeres Binderharz und eine erste und eine zweite Ladungstransportkomponente, wobei eine der Ladungstransportkomponenten eine Terphenyldiamin-Ladungstransportkomponente ist, die ein Isomer von N,N'-Bis(methylphenyl)-N,N'-bis[4-(n-butyl)phenyl]-[p-terphenyl]-4,4"-diamin der Formel (I) umfasst: worin R₁ eine Methylgruppe (-CH₃) in der ortho-, meta- oder para-Stellung ist und R₂ eine Butylgruppe (-C₄H₉) ist, **dadurch gekennzeichnet, dass** die erste Ladungstransportkomponente und die zweite Ladungstransportkomponente verschiedene Isomere von N,N'-Bis(methylphenyl)-N,N'-bis[4-(n-butyl)phenyl]-[p-terphenyl]-4,4"-diamin sind.

2. Bilderzeugungselement nach Anspruch 1, wobei die Ladungstransportkomponente ein Isomer umfasst, ausgewählt aus
i) N,N'-Bis(2-methylphenyl)-N,N'-bis[4-(n-butyl)phenyl]-[p-terphenyl]-4,4"-diamin;
ii) N,N'-Bis(3-methylphenyl)-N,N'-bis[4-(n-butyl)phenyl]-[p-terphenyl]-4,4"-diamin; und
iii) N,N'-Bis(4-methylphenyl)-N,N'-bis[4-(n-butyl)phenyl]-[p-terphenyl]-4,4"-diamin.

3. Bilderzeugungselement nach einem der vorangehenden Ansprüche, wobei das Terphenyldiamin 25 Gew.-% bis 60 Gew.-% der Ladungstransportschicht umfasst, bezogen auf das Gesamtgewicht der Ladungstransportschicht, vorzugsweise 40 Gew.-% bis 50 Gew.-%.

4. Bilderzeugungselement nach einem der vorangehenden Ansprüche, wobei der Binder ausgewählt ist aus der Gruppe bestehend aus Polyestern, Polyvinylbutyralen, Polycarbonaten, Polystyrol und Polyvinylformiaten.

5. Bilderzeugungselement nach Anspruch 4, wobei der Binder ein Polycarbonat, ausgewählt aus der Gruppe bestehend aus Poly(4,4'-isopropyliden-diphenylcarbonat), Poly(4,4'-diphenyl-1,1'-cyclohexan-carbonat), oder eine Polymermischung davon ist.

6. Bilderzeugungselement nach Anspruch 1, wobei die Gesamtdicke der Ladungstransportschicht 10 µm bis 100 µm, vorzugsweise 20 µm bis 60 µm beträgt.

7. Bilderzeugungselement nach Anspruch 1, umfassend ein Substrat, eine optionale leitfähige Schicht, eine optionale Lochblockierungsschicht, eine optionale Klebstoffschicht, eine ladungserzeugende Schicht und die wenigstens eine Ladungstransportschicht,
wobei die Ladungstransportschicht eine untere Schicht und eine obere Schicht umfasst; wobei die untere und obere Schicht jeweils ein polymeres Binderharz und ein Terphenyldiamin der Formel I umfasst; und
wobei die untere Schicht 30 Gew.-% bis 50 Gew.-% des Terphenyldiamins umfasst und die obere Schicht 0 Gew.-% bis 45 Gew.-% des Terphenyldiamins umfasst, wobei die obere Schicht eine niedrigere Konzentration des Terphenyldiamins aufweist als die untere Schicht.

8. Bilderzeugungselement nach Anspruch 7, wobei das Trägersubstrat, welches optional eine leitfähige Oberflächenschicht umfasst, ausgewählt ist aus der Gruppe bestehend aus Kupfer, Messing, Nickel, Zink, Chrom, Edelstahl, leitfähigen Kunststoffen, leitfähigen Kautschuken, Aluminium, halbtransparentem Aluminium, Stahl, Cadmium, Silber, Gold, Zirconium, Niob, Tantal, Vanadium, Hafnium, Titan, Wolfram, Molybdän, Indium, Zinn und Metalloxiden.

9. Verfahren zum Erzeugen eines Bildes, umfassend:
Erzeugen eines elektrostatischen Latentbilds auf einem Bilderzeugungselement;
Entwickeln des Latentbildes; und
Überführen des entwickelten elektrostatischen Bildes auf ein geeignetes Substrat;
wobei das Bilderzeugungselement eine Ladungstransportschicht aufweist, die erste und zweite Ladungstransportkomponenten umfasst, wobei eine der Ladungstransportkomponenten ein Terphenyldiamin mit der Struktur der Formel (I) ist:
worin R₁ eine Methylgruppe in der ortho-, meta- oder para-Stellung ist und R₂ eine Butylgruppe ist, wobei die erste Ladungstransportkomponente und die zweite Ladungstransportkomponente verschiedene Isomere von N,N'-Bis(methylphenyl)-N,N'-bis[4-(n-butyl)phenyl]-[p-terphenyl]-4,4"-diamin sind.

10. Verfahren zum Herstellen eines Bilderzeugungselements nach Anspruch 1, in welchem ein Substrat mit einer Beschichtungszusammensetzung beschichtet wird, die das Harz, die Terphenyldiaminisomere und ein Lösungsmittel, in welchem das Harz löslich ist, umfasst, und die Zusammensetzung getrocknet wird.

## Revendications

1. Élément d'imagerie comprenant au moins une couche de transport de charge comprenant une résine de liaison polymère et un premier et un deuxième composant de transport de charge, dans lequel l'un des composants de transport de charge est un composant de transport de charge à base de terphényl diamine composé d'un isomère de N,N'-bis(méthylphényl)-N,N'-bis[4-(n-butyl)phényl]-[p-terphényl]-4,4"-diamine de Formule (I) : dans laquelle R₁ est un groupe méthyle (-CH₃) dans la position ortho, méta, ou para et R₂ est un groupe butyle (-C₄H₉), **caractérisé en ce que** le premier composant de transport de charge et le deuxième composant de transport de charge sont des isomères différents de la N,N'-bis(méthylphényl)-N,N'-bis[4-(n-butyl)phényl]-[p-terphényl]-4,4"-diamine.

2. Élément d'imagerie selon la revendication 1, dans lequel le composant de transport de charge comprend un isomère choisi parmi
(i) la N,N'-bis(2-méthylphényl)-N,N'-bis[4-(n-butyl)phényl]-[p-terphényl]-4,4"-diamine ;
(ii) la N,N'-bis(3-méthylphényl)-N,N'-bis[4-(n-butyl)phényl]-[p-terphényl]-4,4"-diamine ; et
(iii) la N,N'-bis(4-méthylphényl)-N,N'-bis[4-(n-butyl)phényl]-[p-terphényl]-4,4"-diamine.

3. Élément d'imagerie selon une quelconque revendication précédente, dans lequel la terphényl diamine compose de 25 pour cent en poids à 60 pour cent en poids de la couche de transport de charge sur la base du poids total de la couche de transport de charge, préférablement de 40 pour cent en poids à 50 pour cent en poids.

4. Élément d'imagerie selon une quelconque revendication précédente, dans lequel le liant est choisi parmi le groupe consistant en des polyesters, des poly(butyrals de vinyle), des polycarbonates, un polystyrène, et des poly(formates de vinyle).

5. Élément d'imagerie selon la revendication 4, dans lequel le liant est un polycarbonate choisi parmi le groupe consistant en le poly(diphényl carbonate de 4,4'-isopropylène), le poly(carbonate de 4,4'-diphényl-1,1'-cyclohexane), ou un mélange polymérique de ceux-ci.

6. Élément d'imagerie selon la revendication 1, dans lequel l'épaisseur totale de la couche de transport de charge est de 10 µm à 100 µm, préférablement de 20 µm à 60 µm.

7. Élément d'imagerie selon la revendication 1, comprenant un substrat, une couche conductrice facultative, une couche de blocage de trous facultative, une couche adhésive facultative, une couche de génération de charge, et l'au moins une couche de transport de charge,
dans lequel la couche de transport de charge comprend une couche inférieure et une couche supérieure ;
dans lequel les couches inférieure et supérieure comprennent chacune une résine de liaison polymère et une terphényl diamine de Formule (I) ; et
dans lequel la couche inférieure comprend de 30 pour cent en poids à 50 pour cent en poids de la terphényl diamine et la couche supérieure comprend de 0 pour cent en poids à 45 pour cent en poids de la terphényl diamine, la couche supérieure ayant une concentration de la terphényl diamine inférieure à celle de la couche inférieure.

8. Élément d'imagerie selon la revendication 7, dans lequel le substrat support, qui comprend facultativement une couche de surface conductrice, est choisi parmi le groupe consistant en le cuivre, le laiton, le nickel, le zinc, le chrome, l'acier inoxydable, des plastiques conducteurs, des caoutchoucs conducteurs, l'aluminium, un aluminium semi-transparent, l'acier, le cadmium, l'argent, l'or, le zirconium, le niobium, le tantale, le vanadium, le hafnium, le titane, le tungstène, le molybdène, l'indium, l'étain et des oxydes de métal.

9. Procédé d'imagerie, comprenant :
la génération d'une image latente électrostatique sur un élément d'imagerie ;
la révélation de l'image latente ; et
le transfert de l'image électrostatique révélée sur un substrat approprié ;
dans lequel l'élément d'imagerie a une couche de transport de charge comprenant un premier et un deuxième composants de transport de charge, dans lequel l'un des composants de transport de charge est une terphényl diamine ayant la structure de Formule (I) : dans laquelle R₁ est un groupe méthyle dans la position ortho, méta, ou para et R₂ est un groupe butyle, le premier composant de transport de charge et le deuxième composant de transport de charge sont des isomères différents de la N,N'-bis(méthylphényl)-N,N'-bis[4-(n-butyl)phényl]-[p-terphényl]-4,4"-diamine.

10. Procédé de fabrication d'un élément d'imagerie selon la revendication 1, dans lequel un substrat est revêtu avec une composition de revêtement comprenant la résine, les isomères de terphényl diamine et un solvant dans lequel la résine est soluble, et la composition est séchée.
